

# UNITED STATES PATENT OFFICE.

GEORGE M. COLVOCORESSES, OF NEW YORK, N. Y.

## PROCESS OF MANUFACTURING IRON ALLOYS.

1,106,786.

Specification of Letters Patent.

Patented Aug. 11, 1914.

No Drawing.

Application filed June 19, 1913. Serial No. 774,641.

To all whom it may concern:

Be it known that I, GEORGE M. COLVOCORESSES, a citizen of the United States of America, and residing at New York, in the county of New York and State of New York, have invented new and useful Improvements in Processes of Manufacturing Iron Alloys, of which the following is a specification.

10 The main object of the present invention is to provide for the commercial manufacture of an iron alloy and more particularly for the manufacture of a nickel-copper alloy steel directly from the slags which are 15 at present run to waste from furnaces used in the smelting of ores containing iron, nickel and copper as sulfids.

The ores to which I refer are more particularly those which are referred to as 20 nickeliferous pyrrhotite with chalcopyrite and are found most abundantly in the Sudbury District of Ontario, Canada, in other sections of Canada, and in certain districts of the United States and of Norway, and to 25 a lesser extent in other countries. The furnace slags from smelting these ores have heretofore been run to waste or in some cases, used for railroad ballast or road material replacing crushed stone for these 30 purposes, and in a few instances, these slags have been used in the manufacture of cement. Up to the present time none of the experiments which have been made in smelting the slags have resulted in the manufacture 35 of a commercially valuable metallic product.

As examples of the ores from which are obtained the slags which I propose to treat according to my invention, I may mention 40 the following compositions:

|                            | No. 1,<br>basic. | No. 2,<br>medium. | No. 3,<br>silicious. |
|----------------------------|------------------|-------------------|----------------------|
| Iron, Fe.                  | 50%              | 46%               | 40%                  |
| Sulfur, S.                 | 29%              | 25%               | 20%                  |
| Nickel, Ni.                | 1.5%             | 2%                | 2.5%                 |
| Copper, Cu.                | 4%               | 5%                | 1%                   |
| Silica, SiO <sub>2</sub> . | 10%              | 20%               | 32%                  |
| Magnesia, MgO.             |                  |                   |                      |
| Lime, CaO.                 |                  |                   |                      |
| Nickel, Ni.                |                  |                   |                      |

Alumina, Al<sub>2</sub>O<sub>3</sub>} Small varying quantities.

These ores are according to the present commercial practice, roasted to remove a 50 portion of the sulfur and then smelted with

flux in water jacket blast furnaces or in 55 reverberatory furnaces similar to those used in copper smelting, whereby the greater part of the copper and nickel are combined with the sulfur in a matte and a portion of the iron together with small percentage of copper and nickel, a little sulfur and the greater part of the silicon and non-metallic elements are separated out as a slag. By manipulating the charge of the blast or reverberatory furnace in a suitable manner, I 60 can, if desired, produce a "foul slag" that is, one containing more nickel and copper than has been found economical to make in the past and containing also as large a percentage of iron as metallurgically feasible 65 and from this "foul slag" I can produce an iron alloy containing more nickel and copper than in the alloy made from the clean or ordinary slag.

Examples of the slag which I propose to 70 treat are as follows:—

|                                           | No. 1, clean. | No. 2, foul. |
|-------------------------------------------|---------------|--------------|
| Iron, Fe.                                 | 41.40%        | 45.60%       |
| Sulfur, S.                                | 1.50%         | 2.00%        |
| Silica, SiO <sub>2</sub> .                | 30.00%        | 25.00%       |
| Alumina, Al <sub>2</sub> O <sub>3</sub> . | 5.50%         | 5.00%        |
| Magnesia, MgO.                            | 2.00%         | 1.50%        |
| Lime, CaO.                                | 2.50%         | 2.00%        |
| Copper, Cu.                               | 0.25%         | 0.50%        |
| Nickel, Ni.                               | 0.40%         | 1.00%        |

By my process I make an iron-nickel-copper-alloy and a nickel-copper-alloy-steel 85 direct from these slags. I run the slag (preferably in the molten or heated condition) into an iron blast furnace of standard type and similar to those employed in iron smelting or into an electric shaft furnace and 90 there smelt it with coke, limestone, and other flux into a ferro nickel-copper pig, which will also contain a certain amount of impurities and if produced in the coke blast furnace it will also contain sulfur from 1% 95 to 4%. The pig produced from this process, I transfer directly and preferably molten into an electric refining furnace where it is purified by removing the excess silicon, practically all of the sulfur, and so 100 much carbon as may be desired and transformed into a high-grade nickel-copper-alloy-steel containing only such impurities as are usually found in high-grade steels.

The content of nickel-copper will vary in accordance with the slag employed, but in general, the nickel content will be from 0.4 to 4% and the copper from 0.2% to 2%. 5 In case the nickel and copper content is too low additional nickel and copper as such may be added and in case the nickel and copper are in excess more iron may be added to produce the desired alloy, the additional elements being charged in the refining furnace along with the pig.

The slags which are at present on the dumps of the old smelters either run out from slag pots or granulated may be handled in a manner entirely similar to the above, and before smelting they may be briqueted or heated to a molten state in reverberatory furnaces.

Examples of the steel made by my process 20 less from the clean and foul slags above tabularized are approximately as follows:

|             | No. 1. | No. 2. |
|-------------|--------|--------|
| Nickel, Ni. | 1.00%  | 2.20%  |
| Copper, Cu. | .60%   | 1.10%  |
| Iron, Fe.   | 98.15% | 98.60% |
| Carbon, C.  | .25%   | .10%   |

It is not my intention however, to limit my steel to the exact composition mentioned above. The steels made by this process have a great mechanical strength, and are very useful in the arts and industries. Steel #1 is superior to the ordinary carbon steel and steel #2 has the same superior qualities as an ordinary nickel-steel containing the same percentage of nickel as of combined nickel and copper in my steel.

Examples of the qualities of my steel as shown in a test bar, may be cited as follows:

|                       | Steel, No. 1. | Steel, No. 2. |
|-----------------------|---------------|---------------|
| Yield point.          | 51,000        | 60,500        |
| Maximum strength.     | 71,500        | 80,000        |
| Per cent. elongation. | 22.5          | 28.5          |
| Per cent. reduction.  | 62.5          | 63.8          |

The treatment of the iron copper nickel sulfid ores in the past has been of necessity wasteful and improvident since small percentages of the nickel and copper were lost in the furnace slag while in the blast or reverberatory furnace-slag and Bessemer converter-slag, all the iron was fluxed out of the ore and eventually wasted. The Bessemer converter slag is in practice charged back again into the blast furnace and then remelted so that in the present method of smelting all the iron in the ore is eventually lost while by my slag treatment process, all the iron including that which originally adheres to the furnace matte is eventually recovered and forms the nucleus for the manufacture of a valuable alloy steel thoroughly homogeneous in composition and very useful in the arts and industries, and which can be made with commercial profit. I would, therefore, consider that my process is valuable from the

conservation standpoint since it provides a 65 method of utilizing the iron content of the nickel copper ores amounting on the average to 40% of their weight and also the small quantities of nickel and copper which are lost in the present method of treatment. 70 Further; my process is of value as the sale of the alloy steel made from the slag will very considerably increase the profits which are made by the companies now treating the nickel-copper iron ores and will thus tend 75 to permit the extraction and treatment of a lower grade of this ore than can at present be handled with profit.

I have used the term iron alloy in a broad 80 sense to include steel containing various percentages of carbon, the preferred product is an iron, nickel, copper, carbon alloy or a nickel-copper-alloy-steel.

It will be obvious that for economical 85 reasons the different steps of my process may be carried out in different places. For instances, the slag may be smelted at one place and the resultant pig shipped to another place for refining.

What I claim is:—

1. The process of making an iron alloy which consists in smelting a furnace slag containing iron, copper and nickel with suitable fuel and flux to form a copper nickel ferro pig, slagging off most of the non-metallic elements and reducing the metallic oxides contained in the slag and refining the resultant ferro nickel pig to remove the remaining undesirable elements and to regulate the carbon and retaining throughout the process and in combination substantially all the iron, nickel and copper that existed in the original slag.

2. The process of making an iron alloy which includes smelting with suitable fluxes, a furnace slag containing iron, nickel and copper to eliminate the non-metallic elements as silicates and reduce the oxides of said metals to a composite pig of iron, nickel and copper suitable for subsequent refining.

3. The process of making an iron alloy which includes smelting with suitable flux an iron nickel copper slag containing from 20 to 50% iron, from .2 to 2% nickel and from 0.1 to 2% copper, and reducing the metallic oxides to a composite pig of iron, nickel and copper suitable for refining.

4. The process of making a steel alloy which includes simultaneously smelting the oxides of iron, nickel, copper and silica as they occur in a blast or reverberatory furnace slag all in combination with a suitable flux to eliminate the silica and other non metals if present, and to reduce the metallic oxides to a nickel, copper ferro pig and then refining the composite pig and forming a nickel-copper-alloy-steel.

5. The process of making a steel alloy

which comprises smelting an iron, nickel, copper slag containing approximately from 20 to 50% of iron, from .2 to 2% of nickel and from .1 to 2% copper so as to reduce the 5 metallic compounds to a composite pig of iron, nickel and copper and then refining the pig at a sufficiently high temperature to

produce a nickel-copper-steel alloy containing approximately from .2 to 2% copper, from .4 to 4% nickel and up to 1% carbon.

GEORGE M. COLVOCORESSES.

Witnesses:

ROBT. S. ALLYN,  
E. BRADFORD.